

## UNITED STATES PATENT OFFICE.

EDWARD A. NILL AND FREDERICK C. ACKER, OF CLEVELAND, OHIO, ASSIGNEES, BY DIRECT AND MESNE ASSIGNMENTS, OF ONE-THIRD TO PEARL E. SELBY, OF PORTSMOUTH, OHIO, AND TWO-THIRDS TO J. R. DALL, OF NORWALK, OHIO.

## LUBRICANT.

No Drawing.

Application filed August 31, 1922. Serial No. 585,527.

This invention relates to improvements in semi-solid lubricants.

The general object of the invention is to make a lubricant of a semi-solid nature having a high degree of lubricating value and containing no non-lubricating elements such as are frequently used to effect a combination of the elements, solidification, etc., but wherein all the elements contribute to 10 the lubricating value.

A further object is to make such a lubricant of materials easily obtained and by a simple effective process.

A still further object is to produce such a 15 lubricant which shall not be impaired by low temperatures.

In the making of semi-solid lubricants, or greases, the common practice has been to mix mineral oils with soaps of lime, soda, 20 alumina, lead, etc., or to include some inert substance such as clay or talc. It is obvious that such mixtures have elements deleteriously affecting the lubricating properties and do not have ideal lubricating 25 values on account of the readiness of the saponified base to separate from the oil. Also, in such greases, there is usually present a free mineral or organic material, resulting in solidification or "caking" of the 30 material when in the bearings.

To overcome the above mentioned difficulties, we desire to use only materials all of 35 which contribute to the lubricating character of the mixture. To this end, we desire 40 to unite lubricating oils of a hydro-carbon character with animal or vegetable oils in such a manner as to have a complete mixture and satisfactory solidification and avoid any tendencies to separate even when in use.

According to the method of making the lubricant of our invention, we are enabled 45 to have solidification and composite union of liquid petroleum, or fatty lubricating oil or mixtures thereof with the addition of hydrogenated fatty oils, such as for example, hydrogenated castor oil, corn, cotton seed, soya bean, coconut, sesame, lard, cod and other hydrogenated fatty oils. We 50 find that we may use for hydrogenation any vegetable or animal oil of an unsaturated nature including fish oils and the like, which

may be broadly termed oils of "marine animal" origin.

The lubricating value of our composition is particularly enhanced by a percentage of castor oil, such, for example, as 3% to 25%. Such an oil greatly reduces the coefficient of friction, under heavy load and improves the wearing properties of the compound. The same is true of rape seed oil. An example of a combination of oils which may be given as having proven to be very satisfactory for a semi-solid lubricant such as are used for automobile gears, bearings 60 and the like, as well as in places where such semi-solid lubricants are used may be as follows:—

80% by volume—neutral oil. This may be 500 seconds Saybol universal at 100° 70 Fahrenheit viscosity Texas petroleum.

15% by volume—hydrogenated organic oil, preferably castor oil.

5% castor oil.

Following the discovery that combinations such as above outlined comprise compounds having greater lubricating value than those produced by using soaps, it has been found that to make such lubricants in a practical and efficient fashion, and cause 80 a complete and uniform uniting of the compound, refrigeration may be employed to effect solidification as will be presently described.

Our preferred method of uniting oils 85 which do not of their nature form a satisfactory union or compound is as follows:—

The various ingredients having been measured out, are melted together at a temperature slightly in excess of the melting point 90 of hardened fat or other organic oil and the mass is uniformly mixed by means of mechanical agitation, while maintaining a melting temperature. The mixed compound is then allowed to flow upon a revolving cylinder or chilled roll whose surface is maintained at a very low temperature by means of circulating brine chilled by any well-known method of refrigeration. The warm liquid of the compound flowing over this chilling cylinder, hardens to a semi-solid 100 state in a continuously moving thin transparent layer which is removed by well known methods and caused to fill suitable

containers. We find that the temperature of the brine and correspondingly the chilling cylinder may be kept at from zero centigrade to minus 18° centigrade, depending upon the grade of lubricant being made.

By this method, the united ingredients do not melt and later separate under warm weather conditions, neither do they unduly harden and lose their value as lubricants under temperatures approximating those at which they were originally cooled.

From the foregoing specification, it will be seen that by our invention, we have united lubricating elements not heretofore successfully used in compounds of this character. We have thus been enabled to produce a lubricant which experience has demonstrated is very satisfactory in use and avoids the difficulties of previous lubricants of this general character. It will be seen that the process by which the ingredients are compounded is a very simple one.

Having thus described our invention, what we claim is:

1. A lubricant consisting of four parts neutral petroleum oil and one part consisting

of both fatty lubricating oil and hydrogenated fatty oil, whereby a semi-solid homogeneous mixture is obtained.

2. A lubricant consisting of a hydrocarbon oil, relatively small proportions of castor oil, an unsaponified hydrogenated fatty oil in proportion greater than that of the castor oil.

3. A semi-solid lubricant consisting of ingredients in substantially the following proportions:—neutral oil 80%; hydrogenated oil 15%; castor oil 5%.

4. A lubricant comprising a mechanical mixture of approximately four parts, neutral petroleum oil, one part of both castor oil and a solidifying agent in the form of a hydrogenated fatty oil.

5. A semi-solid lubricant comprising a mixture, the major portion of which is a neutral petroleum oil, and hydrogenated castor oil serving as a solidifier.

In testimony whereof, we hereunto affix our signatures this 29th day of August, 1922.

EDWARD A. NILL.  
FREDERICK C. ACKER.

containers. We find that the temperature of the brine and correspondingly the chilling cylinder may be kept at from zero centigrade to minus 18° centigrade, depending upon the grade of lubricant being made.

By this method, the united ingredients do not melt and later separate under warm weather conditions, neither do they unduly harden and lose their value as lubricants 10 under temperatures approximating those at which they were originally cooled.

From the foregoing specification, it will be seen that by our invention, we have united lubricating elements not heretofore 15 successfully used in compounds of this character. We have thus been enabled to produce a lubricant which experience has demonstrated is very satisfactory in use and avoids the difficulties of previous lubricants 20 of this general character. It will be seen that the process by which the ingredients are compounded is a very simple one.

Having thus described our invention, what we claim is:—

25 1. A lubricant consisting of four parts neutral petroleum oil and one part consisting

of both fatty lubricating oil and hydrogenated fatty oil, whereby a semi-solid homogeneous mixture is obtained.

2. A lubricant consisting of a hydrocarbon oil, relatively small proportions of castor oil, an unsaponified hydrogenated fatty oil in proportion greater than that of the castor oil.

3. A semi-solid lubricant consisting of ingredients in substantially the following proportions:—neutral oil 80%; hydrogenated oil 15%; castor oil 5%.

4. A lubricant comprising a mechanical mixture of approximately four parts, neutral petroleum oil, one part of both castor oil and a solidifying agent in the form of a hydrogenated fatty oil.

5. A semi-solid lubricant comprising a mixture, the major portion of which is a neutral petroleum oil, and hydrogenated castor oil serving as a solidifier.

In testimony whereof, we hereunto affix our signatures this 29th day of August, 1922.

EDWARD A. NILL.  
FREDERICK C. ACKER.

#### CERTIFICATE OF CORRECTION.

Patent No. 1,617,077.

Granted February 8, 1927, to

EDWARD A. NILL and FREDERICK C. ACKER.

It is hereby certified that the above numbered patent was erroneously issued by direct and mesne assignments of one-third to Pearl E. Selby, of Portsmouth, Ohio, and two-thirds to J. R. Dall, of Norwalk, Ohio, whereas said Letters Patent should have been issued one-third to the inventor said Acker, one-third to Pearl E. Selby, of Portsmouth, Ohio, and one-third to J. R. Dall, of Norwalk, Ohio, as assignees by direct and mesne assignments of the entire interest in said invention, as shown by the records of assignments in this office; and that the said Letters Patent should be read with this correction therein that the same may conform to the record of the case in the Patent Office.

Signed and sealed this 26th day of April, A. D. 1927.

Seal.

M. J. Moore,  
Acting Commissioner of Patents.

**CERTIFICATE OF CORRECTION.**

**Patent No. 1,617,077.**

**Granted February 8, 1927, to**

**EDWARD A. NILL and FREDERICK C. ACKER.**

**It is hereby certified that the above numbered patent was erroneously issued by direct and mesne assignments of one-third to Pearl E. Selby, of Portsmouth, Ohio, and two-thirds to J. R. Dall, of Norwalk, Ohio, whereas said Letters Patent should have been issued one-third to the inventor said Acker, one-third to Pearl E. Selby, of Portsmouth, Ohio, and one-third to J. R. Dall, of Norwalk, Ohio, as assignees by direct and mesne assignments of the entire interest in said invention, as shown by the records of assignments in this office; and that the said Letters Patent should be read with this correction therein that the same may conform to the record of the case in the Patent Office.**

**Signed and sealed this 26th day of April, A. D. 1927.**

**M. J. Moore,  
Acting Commissioner of Patents.**

**Seal.**